

# UNITED STATES PATENT OFFICE.

ANDREW TURNBULL, OF LIVERPOOL, AND THOMAS BURNELL CARMICHAEL, OF WATERLOO, NEAR LIVERPOOL, ENGLAND; SAID CARMICHAEL ASSIGNOR TO SAID TURNBULL.

## TANNING MEDIUM.

1,288,458.

Specification of Letters Patent. Patented Dec. 17, 1918.

No Drawing.

Application filed July 16, 1917. Serial No. 180,877.

To all whom it may concern:

Be it known that we, ANDREW TURNBULL and THOMAS BURNELL CARMICHAEL, subjects of the King of Great Britain, residing at Liverpool, and Waterloo, near Liverpool, respectively, both in the county of Lancaster and Kingdom of England, have invented certain new and useful Improvements in Tanning Mediums, of which the following is a specification.

In the process of converting hides and skins into leather, if the solutions of the tanning agents employed at the commencement be too strong, the outside fibers quickly become tanned and more or less impervious to the penetration of the tanning agent, so that the inside fibers either remain untanned or become only lightly tanned. On the other hand, by the usual process beginning with very weak liquors and continuing with liquors of gradually increasing strengths, the time spent in the operation is very considerable and there is a great waste of material.

Now, our invention is designed to enable a comparatively strong solution or solutions of very varying strength, to be used and yet avoid these evils. At the same time the resultant leather is fuller and otherwise greatly improved from absorption of the special material used and the more thorough fixation of the tanning agent.

Our process consists in preparing and utilizing the jellies or colloidal liquors which are formed when starch granules are heated to a suitable temperature with aqueous solutions of vegetable, artificial or mineral tanning agents. For this purpose we use starch, or natural products containing starch as their principal ingredient with a minimum of gluten, such as ordinary laundry starch, farina, flour from sago, arrowroot, tapioca, cassava, manioc, &c.

When starch is mixed with an aqueous liquid and the temperature raised to 180° F., the starch granules, as is well known, swell and imbibe the liquid to form a jelly or colloidal liquor. If the aqueous liquid employed be an extract of vegetable tannins, these dissolve in the jelly and on cooling remain in a state of whole or partial solution. This colloidal condition of the tanning

agent is the best suited for quick and even penetration of hide fibers. Somewhat similar colloidal tanning liquors can be prepared with artificial tanning agents such as neradol, &c. If the aqueous liquid employed be a strong solution of a basic chrome salt, such as is used for making liquors for chrome leather tannage, a clear bluish green colored jelly is obtained, with extraordinary power of quick and even penetration. Further, the addition of a suitable vegetable tanning material to the bluish green chrome jelly, causes the formation of a more or less brown jelly which readily penetrates hide fiber yielding an excellent combination leather of chrome and vegetable tanning. The clear jelly formed by basic aluminium salts yields a very satisfactory full white leather, which readily forms a good combination leather when suitably treated with vegetable tannins.

By treating properly prepared "pelt," which is hide or skin freed from hair and rough flesh, by the preliminary processes in a tannery, with one or other of the above described jellies or colloidal liquors, in "layer" (laid flat), or in suspension in pits or by drumming, the tanning agents in their colloidal condition with starch, quickly and evenly penetrate the pelt fibers, converting them into leather with specially desirable qualities of fullness, substance, firmness and weight.

The strengths of the tanning agents employed, and the proportion and quality of starch used in preparing the above described jellies or colloidal liquors, may be varied greatly, and the jellies or colloidal liquors may be utilized until nearly exhausted or they may be concentrated by evaporation or addition of more starch or tanning agent as desired. The colloidal starch helps to equalize the strength throughout the mass, and appears to form with the tanning agent a true colloid. In this condition the tanning agent is presented to the fibers with the astringency sufficiently reduced to avoid what is technically known as "case-hardening" being just so that it is absorbed in regulated quantity by all the fibers even to the center of the thickest hide. In addition, when the resultant leather is dried, the

tanning materials are more thoroughly fixed against the solvent action of water than is the case with ordinary leather.

In order to more fully describe the nature 5 of our invention, we append by way of illustration four cases of its practical application.

*Vegetable tannage.*

10 In a copper steam-jacketed pan, to 500 gallons old blended tan-liquor, such as is commonly used in a mixed sole leather tannage, strengthened to 125° barkometer with a suitable tanning extract such as lightly bisulfited quebracho, carefully stir in 250 lbs. finely powdered starch, and with constant stirring quickly raise the temperature to 180° F. Keep at this temperature for fifteen minutes and cool. The jelly is put into 15 an ordinary tan-pit and delimed sole leather butt pelt is laid flat grain down in it, using wooden plungers to push the butts down and having strings attached to two corners for convenience in removing. There is no need 20 for frequent handling to insure even color, but after two days it is advisable to utilize the partly spent jelly for a fresh pack of butts, and to put the partly tanned butts forward into a fresh jelly from which they need 25 not be moved for four days, the jelly from which they are then taken being used for the pack of butts which follows them. The butts are thus moved forward until even the thickest parts on cutting show evenly colored 30 through, which seldom requires more than three weeks. Sufficient acetic or other suitable organic acid should be added to the tan-pits to insure reasonable plumpness and firmness according to the character of the 35 leather required. When quite colored through the butts may be suspended in 150° barkometer warm chestnutwood extract liquor to increase the solidity and weight, before finishing for sole leather in the usual 40 way. Dressing leather would not require 45 this final treatment.

*Chrome tannage.*

In a copper steam-jacketed pan dissolve 50 500 lbs. chrome alum in 350 gallons warm water, and slowly add with constant stirring 65 lbs. soda ash dissolved in 25 gallons warm water. With the temperature not above 100° F. stir in 250 lbs. finely powdered 55 starch and with constant stirring quickly raise the temperature to 180° F. Keep at this temperature for fifteen minutes and cool. This jelly is put into an ordinary tan-pit and delimed sole leather butt pelt is laid 60 flat grain down in it, using wooden plungers to push the butts down and having strings attached to two corners for convenience in removing. Within two days the butts will be found evenly chromed through, but it is 65 advantageous to give about a week for sole

or belting leather to get the requisite fullness.

*Chrome combination tannage.*

In the basic chrome liquor described above 70 under Chrome tannage, before adding the starch dissolve 750 lbs. plantation gambier in the chrome liquor, then add the starch and proceed as before. Heavy butts require considerably longer in this chrome 75 vegetable tannin combination jelly to color evenly through. Somewhat similar combination leather can be obtained by following the above described chrome tannage with a starch gambier tannage. 80

*Alum tannage.*

In a copper steam-jacket pan dissolve 250 lbs. aluminium sulfate in 350 gallons warm water, and slowly add with constant stirring 85 30 lbs. soda ash dissolved in 25 gallons warm water. With the temperature not above 100° F. stir in 250 lbs. finely powdered starch, and with constant stirring quickly raise the temperature to 180° F. 90 Keep at this temperature for fifteen minutes and cool. This jelly is put into an ordinary tan-pit and delimed butt pelt of thick substance laid flat in it for two or more days will be found evenly penetrated, a fuller 95 leather being obtained by giving the longer time. This leather suitably treated with starch gambier jelly or strong liquor of gambier gives an excellent alum vegetable tannin combination leather. 100

In the appended claims the word starch will be employed as denoting ordinary starch or materials consisting mainly of starch in which the degree of hydrolysis is but low. When potato starch for instance, 105 is subjected to conditions leading to hydrolysis, the first result will be the disruption of the starch cells; this may be effected by warming with water to 180° F. The next result will be the production of the so-called 110 "soluble starch." So far each of these products, namely, gelatinized starch and "soluble starch" are still "starch" in the strict chemical sense of the word, and as the word is employed in the appended claims; each 115 product gives the characteristic starch reaction with iodin. If now the starch is further subjected to hydrolytic influences, the "starch reaction" will gradually decrease in intensity and the material will run through 120 a whole gamut of degradational changes until finally dextrin and dextrose are obtained. It will be understood therefore that the word "starch" is hereafter employed to denote bodies in which such hydrolytic action is but 125 slight, which bodies form jellies with the tanning agent, as distinguished from the bodies such as dextrin and dextrose at the other end of the above described gamut of changes. 130

We declare that what we claim is:—

1. A process of preparing a tanning medium which consists in combining a tanning agent with starch including the step of gelatinizing the starch by heating it to about 180° F. in presence of water.
2. An improved tanning medium consisting of a tanning agent plus gelatinized starch.
- 10 3. An improved tanning medium consisting of a mineral tanning agent plus gelatinized starch.
4. An improved tanning medium consist-

ing a chrome tanning agent plus gelatinized starch.

- 15 5. As a composition of matter, a colloidal jelly-like composition containing a tanning agent and gelatinized starch.

In witness whereof, we have hereunto signed our names this 26th day of June 1917, 20 in the presence of two subscribing witnesses.

ANDREW TURNBULL.

THOMAS BURNELL CARMICHAEL.

Witnesses:

W. P. THOMPSON,  
CHAS. LESLIE.